

Dec. 24, 1929.

H. A. TEEPLE

1,740,883

SHINGLE

Filed May 19, 1927

*Fig. 1.*



*Fig. 2.*

Inventor  
H.A.Teeple,

By Bernard J. Farney  
Attorney

## UNITED STATES PATENT OFFICE

HARVEY A. TEEPLE, OF GREENE, IOWA

## SHINGLE

Application filed May 19, 1927. Serial No. 192,602.

The present invention consists of a shingle having for an object the provision of a compact durable shingle which may be flexed under pressure to facilitate laying the shingle and in order to conform to building conformations or irregularities such as are encountered at times in shingling roofs, walls, etc.

Another object of the invention is to provide a water-proof and fire-proof shingle which may be subjected to heat in excess of 200° F. without disintegration or deterioration and without relieving the shingle of any of the desirable characteristics common to shingles of standard construction.

15 A further object of the invention is to provide a shingle of customary contour which may be manufactured at a very low cost and which will last for an indefinite period of time.

20 A still further object of the invention is to provide a novel method of making shingles out of standard weather-proof materials, the method being exceedingly simple to permit expeditious manufacture of the shingles at a minimum cost.

25 Other objects of the invention will be apparent from the following description of the present preferred form of the invention, taken in connection with the accompanying drawings, wherein

Figure 1 is a plan view of a shingle constructed in accordance with the present invention; and,

Figure 2 is a transverse sectional view of 30 the same.

The device of the present invention comprises a body or core 3 preferably made of metal, such as tin or sheet steel, the body or core being of any desired size, but being of a thickness which will permit it to be freely flexed under pressure. The core is enveloped in a bituminous casing 4, which is applied to the core by a particular method which will be hereinafter set out. The casing in the 40 present instance is preferably formed from a composition of rubber, pitch and sand. Attention is directed to the fact that the core is completely enclosed and if desired, the shingle when finished may be tapered toward 45 one end.

The method employed in making the present shingle consists in advancing the core through an applicating machine which contains a mixture of rubber, sand and pitch. This mixture is agitated in the presence of 55 heat, so as to thoroughly mingle the rubber, sand and pitch. From the applicating machine the shingles are passed through rollers which compress the composition on the core and in view of the inherent cementitious 60 character of the composition, the latter is caused to adhere to the surfaces and edges of the core, so as to form an envelope for the latter. From the rollers the shingles are ejected on to a conveyor belt which transports the shingles to a suitable storage place.

65 The composition is preferably composed of from 2 to 10 per cent rubber; from 10 to 20 per cent pitch; and from 40 to 80 per cent sand. This composition is water- and fire-proof in addition to providing an excellent 70 wearing surface capable of withstanding the elements and when applied to a core in accordance with the present invention, will not disintegrate or deteriorate in any way when subjected to heat, even in excess of 200° F. In addition, the shingles may be handled with facility by workmen and may be stored for an indefinite period of time before being used 75 without any deterioration whatsoever.

80 It is, of course, to be understood that the shingle is susceptible of a variety of uses and that various changes may be made therein within the scope of the present claim, it being essential, however, that the shingle be flexible 85 and both fire-proof and water-proof.

I claim:

85 A shingle including a metal core, and a casing, composed of rubber, pitch and sand, enveloping the core.

90 HARVEY A. TEEPLE.